

2,907,654

## HIGH TEMPERATURE TANTALUM-COLUMBIUM BASE ALLOYS

Rudolf H. Thielemann, Palo Alto, Calif., assignor to Sierra Metals Corporation, a corporation of Delaware

No Drawing. Application July 1, 1957  
Serial No. 668,892

6 Claims. (Cl. 75—174)

This invention relates to a tantalum-columbium-chromium base metal alloy, and particularly to one such alloy which contains chromium and tungsten, which alloy has excellent corrosion resistance and possesses great mechanical strength at temperatures of the order of 2000° F. and higher.

Important features of the alloy of this invention are (1) that it may be hot-worked, (2) is highly resistant to oxidation and other forms of corrosion of temperatures up to about 2000° F. and higher, and (3) possesses great mechanical work strength at these elevated temperatures. As a result, this alloy may be used as blades, vanes and other parts of high temperature gas turbine engines. Other important uses of the alloy of this invention are that it may be used as exhaust valves and manifolds in internal combustion engines, in heat exchangers, and as linings for retorts and container vessels used in the chemical and metallurgical industries.

The prior art high temperature, high strength base metal alloys such as the nickel and/or cobalt base metal alloys which have been used as blades, vanes and other parts of high temperature gas turbine engines, have a maximum operating temperature of about 1500° F. For example, a common nickel-cobalt base metal alloy which incorporates molybdenum as a constituent is for all practical purposes non-utilizable as a structural member in a gas turbine engine if the metal temperature significantly exceeds about 1500° F. because of the strength and oxidation resistance limitations of such an alloy above this temperature.

In contrast, the alloy of this invention when used as a blade or vane in a high temperature gas turbine engine can be operated at markedly higher temperatures than was possible heretofore, and the performance of the gas turbine engine is improved in that the total thrust is increased and the amount of fuel consumed per pound of thrust per hour is decreased.

An alloy of this invention is particularly resistant to oxidation and has high strength at elevated temperatures of about 2000° F. and higher, so as to be suitable for use in forming liners for retorts and container vessels used in the chemical and metallurgical industries.

The metal alloy of this invention is comprised, by weight, of approximately 5 percent to 20 percent of chromium, 2 percent to 25 percent of tungsten, and the balance, essentially a mixture of tantalum and columbium, the amount of tantalum in the mixture of tantalum and columbium being from about 10 percent to 95 percent, and the balance of the mixture being essentially columbium. The proportions of the preferred alloys of this invention are, by weight, approximately 10 percent to 20 percent of chromium; 5 percent to 15 percent of tungsten, and the balance, essentially a mixture of tantalum and columbium, the amount of tantalum in the mixture being from about 30 percent to 95 percent, and the balance of the mixture being essentially columbium.

It is important to note that in the past it has been the general understanding that the metals tantalum and

2

columbium are substantially equivalent. I have found that this is not the case in the present invention. Thus, for example, I have found that a relatively small amount of chromium as an alloying constituent with columbium and tungsten renders the resulting columbium-tungsten-chromium metal alloy too brittle to be of any practical use. On the other hand, I have discovered that when tantalum is alloyed with columbium and tungsten in the proportions specified above, then materially larger proportions of chromium can be incorporated, resulting in the new tantalum-columbium-tungsten-chromium alloy of this invention having unexpected, improved properties as indicated above. These properties are not achieved with a columbium-tungsten-chromium metal alloy.

15 To achieve the optimum desired properties in an alloy of the present invention, the impurities named below preferably should be held to the following approximate limits by weight. The carbon content in the final alloy preferably should be no more than 0.5 percent; the oxygen content, no more than 0.8 percent, as determined by an increase on ignition technique; the nitrogen content, no more than 0.2 percent; and the iron content, no more than 5 percent.

20 The following are examples of the preparation and test results of the tantalum-columbium-chromium-tungsten metal alloy of this invention:

### Example 1

30 An ingot of a tantalum-columbium-chromium-tungsten metal alloy composition containing by weight 15 percent of chromium, 15 percent of tungsten, 3.5 percent of columbium and the balance, essentially tantalum, was prepared by arc melting an electrode of tantalum to which 3.5 percent columbium, 15 percent tungsten and 15 percent chromium were added. This may be accomplished by pressing a uniform powder mix of tantalum, columbium, chromium and tungsten in the above proportions in the form of bars under a pressure of about 50 tons per square inch, sintering the pressed bars under a vacuum condition of about 1 micron for a period of about 3 hours, and then arc melting the sintered bars under a vacuum condition of about 5 microns or less.

35 The arc melted alloy of this example was tested for 45 oxidation resistance in moving air at about 2000° F. for twenty-four hours. Its resistance to oxidation was about 700 times greater than the resistance to oxidation of substantially pure columbium.

40 The test procedure for oxidation resistance was comprised of preparing test samples of the alloy and the 50 dimensions of such test samples determined prior to subjecting the test samples to the oxidation test conditions. The oxide film which formed on the test samples during testing was removed and the thickness of each 55 tested sample was then measured and compared with the thickness of the test sample prior to submitting it to the test conditions. The same procedure was carried out to determine the oxidation resistance of substantially pure columbium and a comparison made between the 60 oxidation resistance of columbium and the alloy of this example.

65 Test bars (1/4 inch diameter and 3 inches long) were fabricated from the arc melted ingot of this example by hot-working procedure. The 100 hour rupture strength of such bars in moving air at about 2000° F. exceeded 20,000 pounds per square inch (p.s.i.).

### Example 2

70 An ingot of a tantalum-chromium-columbium-tungsten metal alloy composition containing by weight 10 percent of chromium, 10 percent of tungsten, 24 percent of tantalum, and the balance, essentially columbium,

was prepared in the same manner as set forth in Example 1.

The arc melted alloy of this example was tested for oxidation resistance in moving air at about 2000° F. for twenty-four hours in the same manner as set forth in Example 1. The oxidation resistance of the alloy of this example is about 650 times greater than the oxidation resistance of substantially pure columbium.

Test bars (1/4 inch diameter and 3 inches long) were fabricated from the arc melted ingot of this example by hot-working procedure. The test bars had a 100 hour rupture strength in excess of 20,000 p.s.i. at a temperature of about 2000° F. in moving air.

*Example 3*

An ingot of a tantalum-columbium-chromium-tungsten metal alloy composition containing by weight 5 percent of chromium, 25 percent of tungsten, 7.3 percent of tantalum and the balance, essentially columbium, was prepared in the same manner as set forth in Example 1.

The arc melted alloy of this example was tested for oxidation resistance in moving air at about 2000° F. for twenty-four hours in the same manner as set forth in Example 1. The resistance to oxidation of the example of this alloy is about 100 times greater than the oxidation resistance of substantially pure columbium.

Test bars (1/4 inch diameter and 3 inches long) were fabricated from the arc melted ingot of this example by hot-working procedure. Test bars of this example had a 100 hour rupture strength in excess of 20,000 p.s.i. in moving air at about 2000° F.

*Example 4*

An ingot of a tantalum-columbium-chromium-tungsten metal alloy composition containing by weight 20 percent of chromium, 5 percent of tungsten, 7.5 percent of columbium and the balance, essentially tantalum, was prepared in the same manner as set forth in Example 1.

The arc melted alloy of this example was tested for oxidation resistance in moving air at about 2000° F. for twenty-four hours in the same manner as set forth in Example 1. The oxidation resistance of the arc melted alloy of this example is about 800 times greater than the oxidation resistance of substantially pure columbium.

Test bars (1/4 inch diameter and 3 inches long) were fabricated from the arc melted ingot of this example by hot-working procedure. The test bars of this example had a 100 hour rupture strength in excess of 20,000 p.s.i. at a temperature of about 2000° F. in moving air.

*Example 5*

An ingot of a tantalum-columbium-chromium-tungsten metal alloy composition containing by weight 10 percent of chromium, 10 percent of tungsten, 40 percent of columbium, and the balance, essentially tantalum, was prepared in the same manner as set forth in Example 1.

The arc melted alloy of this example was tested for oxidation resistance in moving air at about 2000° F. for twenty-four hours in the same manner described in Example 1. The oxidation resistance of the alloy of this example is about 500 times greater than the oxidation resistance of substantially pure columbium.

Test bars (1/4 inch diameter and 3 inches long) were fabricated from the arc melted ingot of this example by hot-working procedure. The test bars of this example had a 100 hour rupture strength in excess of 20,000 p.s.i. at a temperature of about 2000° F. in moving air.

*Example 6*

An ingot of a tantalum-columbium-chromium-tungsten metal alloy composition containing by weight 5 percent of chromium, 2 percent of tungsten, 18.6 percent of tantalum, and the balance, essentially columbium, was prepared in the same manner as set forth in Example 1.

The arc melted alloy of this example was tested for oxidation resistance in moving air at about 2000° F. for twenty-four hours in the same manner as described in Example 1. The oxidation resistance of the arc melted alloy of this example was about 100 times greater than the oxidation resistance of substantially pure columbium.

Test bars (1/4 inch diameter and 3 inches long) were fabricated from the arc melted ingot by hot-working procedure. The test bars of this example had a 100 hour rupture strength in excess of 20,000 p.s.i. at a temperature of about 2000° F. in moving air.

I claim:

1. A metal alloy which comprises, by weight: 5 percent to 20 percent chromium; 2 percent to 25 percent tungsten; and the balance, essentially a mixture of tantalum and columbium, the amount of tantalum in the mixture of tantalum and columbium being from 10 percent to 95 percent of the mixture, the balance of the mixture being essentially columbium.

2. A metal alloy which comprises, by weight: 10 percent to 20 percent chromium; 5 percent to 15 percent tungsten; and the balance, essentially a mixture of tantalum and columbium, the amount of tantalum in the mixture of tantalum and columbium being from 30 percent to 95 percent of the mixture, the balance of the mixture being essentially columbium.

3. A metal alloy which comprises, by weight: 10 percent chromium; 10 percent tungsten; and the balance, essentially a mixture of tantalum and columbium, the amount of tantalum in the mixture of tantalum and columbium being about 24 percent of the mixture and the balance of the mixture being essentially columbium.

4. A metal alloy which comprises, by weight: 10 percent chromium; 10 percent tungsten; and the balance, essentially a mixture of tantalum and columbium, the amount of columbium in the mixture of tantalum and columbium being about 40 percent of the mixture and the balance of the mixture being essentially tantalum.

5. A metal alloy which comprises, by weight: 5 percent to 20 percent chromium; 2 percent to 25 percent tungsten; and the balance, essentially a mixture of tantalum and columbium, the amount of tantalum in the mixture of tantalum and columbium being from 10 percent to 95 percent of the mixture, the balance of the mixture being essentially columbium, the impurities carbon, oxygen, nitrogen, and iron not exceeding 0.5 percent of carbon, 0.8 percent of oxygen, 0.2 percent of nitrogen, and 5 percent of iron.

6. A metal alloy which comprises, by weight: 10 percent to 20 percent chromium; 5 percent to 15 percent tungsten; and the balance, essentially a mixture of tantalum and columbium, the amount of tantalum in the mixture of tantalum and columbium being from 30 percent to 95 percent of the mixture, the balance of the mixture being essentially columbium, the impurities carbon, oxygen, nitrogen, and iron not exceeding 0.5 percent of carbon, 0.8 percent of oxygen, 0.2 percent of nitrogen, and 5 percent of iron.

References Cited in the file of this patent

UNITED STATES PATENTS

1,588,518 Brace \_\_\_\_\_ June 15, 1926  
1,742,417 Schrobsdorff \_\_\_\_\_ Jan. 7, 1930